

# UNITED STATES PATENT OFFICE.

ERNST FUES, OF HANAU, GERMANY.

## PROCESS OF MANUFACTURE OF A NEW KIND OF PARCHMENT-PAPER.

1,033,757.

Specification of Letters Patent. Patented July 23, 1912.

No Drawing.

Application filed November 20, 1911. Serial No. 661,267.

*To all whom it may concern:*

Be it known that I, ERNST FUES, a subject of the German Emperor, and resident of Hanau-on-the-Main, Germany, have invented certain new and useful Improvements in the Process of Manufacture of a New Kind of Parchment-Paper, of which the following is a specification.

Hitherto only one method of manufacturing parchment paper has been known, which consists in causing concentrated sulfuric acid of from 59° to 61° Baumé (or a concentrated solution of zinc chlorid) to act on paper, papers made from cotton yielding the best results.

I have found that an equally valuable parchment paper can be produced at a very reduced cost and with less danger to the operatives by using very dilute acids, or organic acids, acid salts and such salts as act in a like manner through dissociation in dilute aqueous solution with, or without, the addition of formaldehydes, such substances being employed at a high temperature either in the course of manufacturing the paper, or after it has been made. In the latter case the raw paper which is used in the process can be of varied composition, the so-called imitation parchment paper or greaseproof paper of the so-called Mitscherlich-cellulose made from hard boiled cellulose by grinding to an unctuous or viscous consistency being the most suitable for the purpose in view.

In carrying out the invention the paper is soaked in the aforesaid acid solution and then dried at a temperature of about 100° centigrade for instance on drying cylinders such as are generally used in the manufacture of paper.

If the parchmentizing of the paper is to be effected on the paper machine, the parchmentizing preparation must be of a strength adapted to the amount of moisture in the paper stuff at its point of application.

After the paper has been dried, it possesses, according to its composition and preliminary treatment, a more or less pronounced parchment-like constitution and resistance to the action of water.

Imitation parchment paper or greaseproof paper will be thoroughly parchmentized in accordance with the process I have described. It is conspicuously hard and when viewed through presents an appearance more devoid of structure than has been hitherto obtained by the grinding

process already described. Both these features and its resistance to the disintegrating action of water and its great power of resisting acids and alkalies characterize the 60 parchmentized imitation parchment paper or greaseproof paper as being fully equal in all its valuable properties to genuine sulfuric acid or zinc chlorid parchment paper. For instance ready made dry imitation 65 parchment paper or greaseproof paper can be soaked with a mixture of a solution of about 6 per cent. solution of aluminium sulfate and a 0.6 per cent. solution of formaldehyde, and dried in the usual manner on 70 drying cylinders.

When using sulfuric acid, the parchmentizing can only be obtained when the strength is not less than one tenth of the normal, but with the simultaneous employment of formaldehyde, an acid having 75 1/20th the strength of normal sulfuric acid will suffice to produce a perfect parchmentized paper.

Organic acids exercise on similar raw 80 material a parchmentizing action, which however is less pronounced when formaldehyde is not present than when formaldehyde is used in conjunction with the organic acids. For instance by the action of 85 10 per cent. acetic acid and 0.6 per cent. formaldehyde, a very good parchmentization of the imitation parchment paper or greaseproof paper is obtained following the hereinbefore described mode of treatment. 90 An essential condition is however that the paper should always be treated at a high temperature.

The process is equally effective whether the paper under treatment be sized, or not. 95

Formaldehyde can of course be replaced by its polymerization and addition products, as well as by compounds which, when suitably treated, decompose and liberate formaldehyde and such substances are to be understood as included under the term "formaldehyde" employed in the claims hereof.

The acid remaining in the paper after parchmentization can be washed out or neutralized and rendered harmless in any suitable manner.

The present process differs from the usual parchmentizing processes by means of concentrated sulfuric acid in the following respects: 1. Instead of concentrated sulfuric acid of 59° to 61° Baumé only thoroughly 110 diluted acid substances are employed, such

for instance as a sulfuric acid of not more than 1/10th normal strength. 2. Instead of sulfuric acid, volatile mineral acids such as hydrochloric acid and organic acids are used together with formaldehyde. 3. Acid and other salts which are excluded entirely in the old process of manufacturing parchment paper, such for instance as sulfate of alumina, or bisulfate, can be used in this process with success. 4. Whereas for the manufacture of parchment paper by means of sulfuric acid, pure cotton raw material having as high an absorption power as possible is preferably used, this same raw material, if not subjected to a preliminary treatment, is quite useless for the new process; moreover imitation parchment paper or grease-proof paper is suitable as the raw material for the present process, whereas, on account of its special density and small absorption power, it was totally unfit for the manufacture of genuine parchment paper by means of concentrated sulfuric acid. 5. A high temperature of about 100° centigrade is requisite for carrying out the process.

The new process offers, when compared with that hitherto in use, a considerable improvement as regards economical working, as in consequence of the employment of cheaper raw papers and cheaper chemicals, especially when the paper is produced at one operation on the machine, a considerably cheaper production of parchment paper is obtained as compared with the old process. In addition to this, the present process has the further advantage over the former process that it employs substances which are less

injurious to the health of the operatives than those hitherto used.

I claim:

1. The herein described improvement in the process of manufacturing parchment paper comprising treating suitable raw material with a highly diluted acid solution at a temperature of about 100° C. 40

2. The herein described improvement in the process of manufacturing parchment paper comprising treating suitable raw material with an acid solution and formaldehyde. 45

3. The herein described improvement in the process of manufacturing parchment paper comprising treating suitable raw material with an acid solution and formaldehyde at a temperature of about 100° C. 50

4. Parchment paper produced by treating suitable raw material with a highly diluted acid solution at a temperature of about 100° C. and which paper is relatively hard and adapted to resist in a marked degree the disintegrating action of water, acids and alkalies. 60

5. Parchment paper produced by treating suitable raw material with an acid solution and formaldehyde, said paper being relatively hard, translucent, and not readily affected by water, acids or alkalies. 65

In testimony whereof I have signed my name to this specification in the presence of two subscribing witnesses.

ERNST FUES.

Witnesses:

FRANZ HASLACHER,  
ERWIN DIPPEL.